

No. 788,912.

PATENTED MAY 2, 1905.

J. A. JUST.

PROCESS OF EXTRACTING METALS.

APPLICATION FILED OCT. 7, 1904.



INVENTOR.  
John A. Just  
BY Dickerson, Brown,  
Raegener & Binney ATTORNEYS.

## UNITED STATES PATENT OFFICE.

JOHN A. JUST, OF PULASKI, NEW YORK, ASSIGNOR TO JUST MINING & EXTRACTION CO., OF ROCHESTER, NEW YORK, A CORPORATION OF NEW YORK.

## PROCESS OF EXTRACTING METALS.

SPECIFICATION forming part of Letters Patent No. 788,912, dated May 2, 1905.

Application filed October 7, 1904. Serial No. 227,523.

*To all whom it may concern:*

Be it known that I, JOHN A. JUST, a citizen of the United States, and a resident of Pulaski, Oswego county, State of New York, have invented certain new and useful Improvements in Processes of Extracting Metals, of which the following is a specification, accompanied by a drawing.

This invention relates to processes of extracting metals from their ores, more particularly to the extraction of gold and silver from oxidized and unoxidized ores.

The objects of the invention are to extract all the precious metals in the ore, as gold and silver, more quickly and economically than heretofore; and the invention consists of a new process of extraction, substantially as herein-after fully described and claimed in this specification and as illustrated by the suitable apparatus in the accompanying drawing, in which the figure is a side elevation of suitable apparatus for carrying out the process.

In treating unoxidized sulfid ores containing gold and silver the ore is first roasted, and in carrying out the roasting process the ore should preferably be crushed until it will pass through a sieve of suitable mesh—as, for instance, a sixty-mesh sieve, which has been found of suitable size for extraction. If desired, a somewhat coarser or a finer sieve may be used, according to the apparatus available for circulating the extracting liquid.

In ore that contains approximately ten ounces of gold per ton and two per cent. of silver about five per cent. of sodium chlorid in solution is added to the ore to moisten the ore, and the ore and solution are thoroughly mixed in any suitable manner in order to uniformly distribute the salt throughout the mass, which is then dried, thereby driving off the water and insuring the uniform distribution of the salt throughout all the particles of the mass of ore. With ores having different percentages of gold and silver a suitable percentage of sodium chlorid in solution should be added, and, if desired, calcium chlorid in solution instead of sodium chlorid may be used. The mass of ore is then calcined at a low red heat until the check test shows that the sul-

fids are decomposed, which has been found to take from one to one and a half hours. The check test may be made by taking a small quantity from the roast, washing out the water-soluble chlorids with water, adding strong nitric acid to dissolve any undecomposed sulfids if still present, then filtering and testing the filtrate with hydrochloric acid. If the sulfids are decomposed into chlorids, hydrochloric acid will not give a precipitate in this solution; but if the sulfids are still present nitric acid will decompose them and form silver nitrate, which on the addition of hydrochloric acid will precipitate silver chlorid. When this check test shows the absence of sulfids, the roast is complete, and the ores are ready for further treatment. In the check test strong nitric acid is preferably used, since silver sulfid is soluble therein and silver chlorid is not soluble therein. When the process of chloridizing is complete, the ores are transferred to a suitable vessel, which may be termed the "extraction" vessel, (indicated by A in the drawing.) The mass is first washed with water, which may be led to the vessel A from the water-pipe B, and the washing is continued until substantially all of the soluble salts present are extracted. The vessel A is provided with an outlet-pipe C, having a controlling-cock D, which in this instance is a two-way cock controlling the pipe C, and a branch pipe E, emptying into a suitable tank F. The pipe E, as shown, is provided with a cock g, and another branch pipe, H, having a cock I, leads to the final washing-tank J. In the preliminary washing of the ore the cock D is turned to close the outlet of pipe C and open the pipe E, and the cock g also opens pipe E to the tank F, so that the water entering from the supply-pipe B passes through the tank A, out through pipes C and E to the tank F. The ore is washed until no reaction is obtained on adding potassium ferrocyanid or other suitable reagent, indicating the absence of copper, zinc, and other metals, and no precipitate is obtained on adding calcium chlorid, indicating the practical absence of sulfates.

Suitable means are provided for admitting

chlorin to the tank A, as by means of the chlorin-pipe K, provided with the cock L and leading to the bottom of the tank, as shown. Preferably in the bottom of the tank is arranged a strainer O, and the pipe C communicates with the tank A, preferably below the strainer.

In carrying out my improved process the chloridized ore is chlorinated, and one of the features of my invention consists in chlorinating the chloridized ore in the presence of a medium which is chemically inert to the metals themselves to be extracted, but is capable of dissolving the salts of the said metals. The medium in the presence of which chlorination is carried out is capable of taking up silver chlorid in solution, thus extracting the silver chlorid while the gold is chlorinating, and it also takes up auric chlorid in solution as it is formed in the process of chlorination. I have found that calcium-chlorid solution is a suitable medium. Calcium-chlorid solution is capable of holding the chlorin and of taking up and dissolving auric chlorid and silver chlorid. After the washing has been completed calcium-chlorid solution, acidified with hydrochloric acid and of specific gravity about 1.40, containing about forty-one per cent. of calcium chlorid, is added to the ore in the proportion of between two and a half to three times the weight of the ore. The heavy syrupy calcium-chlorid solution is acidified in order to make it thinner, and thus facilitate filtration. By acidifying the solution its property of dissolving silver chlorid is still further increased. Sufficient calcium-chlorid solution should be added to the ore to provide a layer of solution over the ore of from one-third to one-fourth the depth of the ore. In the process of chlorination the addition of the calcium-chlorid solution saves the chlorin and facilitates the extraction, because the calcium chlorid absorbs the chlorin, and the density of the solution restrains the chlorin from escaping, thereby keeping the chlorin in direct contact with the ore. The chlorin gas diffuses readily, and the gold-chlorid solution as fast as it is formed also diffuses readily throughout the calcium-chlorid solution. The calcium-chlorid solution is also at the same time dissolving the silver chlorid. After the addition of the calcium-chlorid solution as described chlorin gas is passed into the tank through the chlorin-pipe K, during which operation the valve D is turned to close the pipe C and cut off the extractor A from the remainder of the apparatus. The chlorin gas is passed in or into the extractor for several hours or until the mass is saturated and the gold is all in solution, the time depending upon the quantity of gas passing and the amount of gold contained in the ore. When the solution in the extractor A is saturated with chlorin, it may be allowed to stand, or the solution may be filtered directly, accord-

ing to the conditions of extraction—as, for instance, the fineness of the ore. During chlorination the ore is preferably kept agitated, and any suitable well-known means may be provided for agitating the ore in the extractor.

The gold may also be chlorinated by the use of a hypochlorite, preferably calcium hypochlorite or bleaching-powder. The bleaching-powder is incorporated with the roasted and washed ore in the extractor A while still moist, and sufficient water, preferably acidified with hydrochloric acid, is added to combine with the lime base of the calcium hypochlorite, thereby producing nascent chlorin, which acts as a powerful solvent for gold. In the place of the acidified water acidified calcium-chlorid solution may be added, as hereinbefore described. In the reaction calcium chlorid is formed and chlorin is liberated, the stock of calcium chlorid being thus kept up, which more than makes up for any mechanical losses in it which may occur. The excessive calcium chlorid may be used afterward in roasting for chloridizing the ore, especially in mining districts where salt is scarce. The chlorination in a case where hypochlorite is used is allowed to continue for from three to five hours, more or less, according to the quantity of the gold in the roast to be dissolved and taken up in solution.

After chlorination the ore is leached with calcium-chlorid solution of the same strength already described until the leachings as they come from the ore show no milkiness on diluting a small sample with from five to ten times as much water and shaking; the milkiness showing the presence of the silver chlorid and clearness the absence of the same. The gold will be extracted long before the silver, and when the dilution test referred to shows the absence of silver chlorid the silver and gold available have all been extracted. During the step of leaching the valves G and I are closed and the two-way cock D is opened to afford communication between the extractor A and the receiving-tank P. The small samples for testing may be taken from the end of the pipe C or from any other suitable place—as, for instance, at the small cock Q near the tank A.

After leaching the cock D is turned to close the pipe C and open pipe E and the valve I is opened. The mass of ore in the extractor A is then washed with a little water, which may be hot, to recover the calcium chlorid remaining in the mass, which is recovered in the well J as a weak solution of calcium chlorid, which may be used afterward in the roasting process for chloridizing, it being of suitable strength for this operation.

In the receiving-tank P the precious metals are in the form of their chlorids in a calcium-chlorid solution, which solution should be maintained in an acid state, the acidity being

imparted by hydrochloric acid in a limited quantity only. The solution should be rendered decidedly acid to blue litmus-paper.

In carrying out the process a precipitating-tank R is preferably provided, connected to the receiving tank or vat P by the pipe S, provided with the cock T, and after the solution of silver and gold chlorids has been obtained in the vat P it is transferred into the precipitating-tank R. Preferably the precipitating-tank R is provided with means for stirring the contents of the tank, in this instance with an air-pipe U, provided with suitable apertures. The use of air for stirring the contents of the precipitating-tank has the advantage that after the complete precipitation the air rids the solution of its retained hydrogen gas, and the iron being present in a ferrous state will quickly oxidize in the presence of the oxygen of the air which passes through the liquid to the ferric state and becomes harmless. The metallic zinc which I add to the material in the precipitating-tank R is preferably in the form of bars, scrap, or other suitable form, and the currents of air issuing from the apertures in the pipe U will keep the zinc bars, scrap, or other forms clean. The pumping of the precipitate from the tank R is also facilitated by air, which agitates the precipitate and keeps it in suspension.

In order to release the silver chlorid from the calcium-chlorid solution, the latter solution may be somewhat diluted with water, just sufficient for the solution to assume a slight cloudiness or milkiness. This step, while not a necessary one in the carrying out of the process, is preferable, because it hastens the step of precipitation of the metals which follows. A suitable substance or metal is now added to the calcium-chlorid solution which is capable of precipitating the gold and silver in the form of salts, or, preferably, directly in a metallic state. For this purpose I prefer to use a metal—as, for instance, metallic zinc—which will remove the metallic salts in the calcium-chlorid solution in a reduced state or in metallic form.

When a filtered sample from the precipitating vat or receiver R no longer shows milkiness on dilution with water and does not show purple color on the addition of stannous chlorid or give a colored precipitate with hydrogen sulfid, this step of the process of reduction is complete.

According to my new process it will be seen that both silver and gold are obtained at the same time or in one operation, which greatly simplifies the process and prevents losses, more especially of the gold.

As shown, A pipe V leads from the precipitating-tank E to a filter-press W, and the solution containing the precipitate is pumped into the filter-press by means of any suitable pump X. The filter-press W may be of any suitable well-known form or construction

which separates the precipitate from the liquor. The liquor is drawn off from the filter-press W through the pipe Y to the tank Z, which contains the liquid calcium chlorid recovered for future use, thereby contributing to the economic value of this process. A branch pipe a is connected to the pipe Y and provided with a cock b to control the washing-water used for washing the precipitate in the filter-press W.

In the precipitating-tank R the zinc chlorid present in the calcium chlorid is practically equivalent to the amount of metals it has reduced, and while it is a solvent for silver chlorid, though in a lesser degree than calcium chlorid, it does no harm, its quantity being small, and when it has accumulated sufficiently to warrant its removal and recovery it may be readily removed from the calcium-chlorid solution by treating it with an alkaline sulfid, as sodium or calcium sulfid, preferably the latter, since calcium chlorid is then formed, thus adding to the solvent used. Hydrogen sulfid may also be used instead of sodium or calcium sulfid, or the zinc chlorid is preferably precipitated with calcium hydroxid as zinc hydroxid and filtered. The calcium chlorid is thus purified in a simple way and the zinc is recovered. Since the gold is precipitated by ferrous salts, which is the only salt likely to be present in the calcium-chlorid solution and in small quantity at this stage, it is advisable to see that before using the calcium-chlorid solution for fresh extraction all ferrous salts are oxidized to ferric salts. This takes place quickly when the calcium-chlorid solution is exposed to the air—as, for instance, to the air admitted through the pipe U or to atmospheric air. The calcium-chlorid solution containing the ferrous salts is colorless, like water; but when the ferrous salt is oxidized to ferric salt the solution has the color of commercial hydrochloric acid—that is, light greenish yellow. The hydrogen gas evolved by the action of hydrochloric acid on zinc reduces the ferric salt present during the treatment of zinc to the ferrous state. To effect the oxidation of the ferrous salt to ferric salt, if desired, the calcium-chlorid solution, especially in case it has become somewhat diluted in the process of extraction, may be run over shallow heated pans from one to the other, and in this way both concentration and oxidation will be effected.

The metallic precipitate is well washed with water until free from all soluble matter, and it is then dried and may be fused directly, melted, and cast into bars. These bars will contain all the silver and gold of the ore and any copper that may have been in the precipitate.

In case the ore to be treated is a naturally oxidized ore the crushed ore is roasted with about two per cent. of sodium chlorid in solution as may be found necessary, as hereinbe-

fore described and according to the silver contained in the ore to be chloridized. The remainder of the treatment for carrying out my process of extraction of the oxidized ore is the same as already described for unoxidized ore. It has been found that low and high grade ores and oxidized and unoxidized ores may be mixed and the process hereinbefore described carried out so that all the gold and silver is recovered therefrom.

In case it is desired to refine the gold-silver-zinc precipitate obtained by the metallic zinc process the preferable method of refining is by smelting with lead after distilling off the zinc. This method is preferable to the ordinary acid methods, because most of the zinc is thus recovered at once in a form available for use as a precipitant. The dried precipitate is mixed with granulated lead in about 20 the proportions of one to three times the weight of lead to the dried precipitate and charcoal in the proportion of about one-tenth of the weight of the lead. The mixture is placed in a graphite retort and heated, preferably, by means of a gas-furnace. The zinc begins to distil off at about 700° Fahrenheit, and is practically all driven off in four or five hours, the temperature being finally raised to about 1,300° Fahrenheit. Very little gold or 25 silver is thus volatilized, and whatever minute traces that do volatilize remain with the zinc, which is used for subsequent precipitation. The metallic-zinc vapors may be received in a well-cooled condenser, in which most of the 30 zinc condenses as dust, especially while carbon monoxide is being evolved. The material in the retort at the end of the distillation is in appearance like that at the start, but on examination there will be found small shots 35 of bullion all through it and usually several larger masses. The residue may be poured from the retort in a loose state, like sand. It should be mixed with about four or five parts 40 of litharge and melted down on a test, a small amount of iron-filings and silica being added, if necessary. After thorough fusion the slag 45 is skimmed off and the lead cupelled, the resulting litharge being used for the next operation. The bullion after remelting may be 50 cast into bars, which are ready for parting.

If desired, the chlorination may be completed in a separate vessel before the calcium-chlorid solution is added. Furthermore, the solution in the receiving - tank P may be 55 pumped back into the extractor A through pipe e by means of a suitable pump f during the leaching with calcium-chlorid solution, thereby keeping up a continuous circulation until the leaching is completed.

60 This invention may be carried out in any suitable apparatus and in a variety of ways, and therefore I do not limit the invention to the details of the steps of the process.

65 My improved process may also be applied to the extraction of silver alone in case there

is no gold present in the ore, in which case the step of chlorination is omitted and the chloridized ore is treated with calcium-chlorid solution to dissolve the silver chlorid.

I claim, and desire to obtain by Letters Patent, the following:

1. The process of extraction, consisting in extracting precious metals in the form of metallic salts, with acidified calcium-chlorid solution.

2. The process of extraction consisting in extracting precious metals in the form of metallic salts, with acidified calcium-chlorid solution of about 1.40 specific gravity.

3. The process of extracting metals in the form of metallic salts, consisting in chlorinating chloridized ores in the presence of acidified calcium-chlorid solution of about 1.40 specific gravity.

4. The process of extracting precious metals in the form of metallic salts, consisting in chlorinating chloridized ores in the presence of acidified calcium-chlorid solution.

5. The process of extracting metals in the form of metallic salts, from sulfid ores containing gold and silver, which consists in chloridizing the ores, and adding acidified calcium-chlorid solution of about 1.40 specific gravity thereto, chlorinating the mass in the presence of the calcium-chlorid solution, and leaching 95 with an additional amount of said calcium-chlorid solution until the extraction is complete.

6. The process of extracting metals in the form of metallic salts, from sulfid ores containing gold and silver, which consists in chloridizing the ores, washing the same to extract all the water-soluble salts, adding acidified calcium-chlorid solution of about 1.40 specific gravity thereto, chlorinating the mass in the presence of said calcium - chlorid solution, leaching with an additional amount of said calcium-chlorid solution until the extraction is complete, precipitating the gold and silver with a suitable substance, and separating the 100 precipitate from the solution.

7. The process of extracting silver from chloridized ores consisting in first chloridizing the ore, then treating the chloridized ore with acidified calcium-chlorid solution of about 115 1.40 specific gravity.

8. The process of extracting metals in the form of metallic salts, from sulfid ores containing gold and silver, which consists in chloridizing the ores, chlorinating the mass in the presence of acidified calcium-chlorid solution of about 1.40 specific gravity, and leaching with an additional amount of said calcium-chlorid solution until the extraction is complete.

9. The process of extracting metals in the form of metallic salts, from sulfid ores containing gold and silver, which consists in chloridizing the ores, washing the same to extract all the water-soluble salts, chlorinating 125 130

the mass in the presence of acidified calcium-chlorid solution of about 1.40 specific gravity, leaching with an additional amount of said calcium-chlorid solution until the extraction 5 is complete, precipitating the gold and silver, and separating the precipitate from the solution.

10. The process of extracting precious metals from their ores, consisting in treating the chloridized ore with acidified calcium-chlorid solution, precipitating the gold and silver and separating them, and recovering the calcium-chlorid solution for reuse.

11. The process of extracting precious met-

als from their ores, consisting in chlorinating 15 the chloridized ores in the presence of acidified calcium-chlorid solution, precipitating the gold and silver and separating them, and recovering the calcium-chlorid solution for reuse.

In testimony whereof I have signed this specification in the presence of two subscribing witnesses,

JOHN A. JUST.

Witnesses:

E. VAN ZANDT,  
H. L. OBERTEINFFER.